

# United States Patent Office

2,874,074

Patented Feb. 17, 1959

1

2,874,074

## 1,2-SUBSTITUTED IMIDAZOLINIUM SALT AND TREATMENT OF CELLULOSIC FIBROUS MATERIALS THEREWITH

Carl E. Johnson, Westchester, Ill., assignor to National Aluminate Corporation, Chicago, Ill., a corporation of Delaware

No Drawing. Application May 8, 1956  
Serial No. 583,366

21 Claims. (Cl. 117—139.5)

This invention relates to the chemical treatment of fibrous materials, such as textiles and paper, whereby useful properties are imparted thereto. Particularly, it relates to treating textiles with new chemical softening agents, lubricants and water repellent agents. In another embodiment the invention is concerned with new and valuable chemical compositions.

It is an object of the invention to provide new and useful softeners and lubricants for fibrous materials such as textiles and paper.

A further object is to provide textile softeners which are relatively non-toxic and do not tend to yellow bleached fabrics. Other objects will appear hereinafter.

It has been found that fibrous materials when treated with a colloidally dispersible 1,2-substituted imidazolinium salt which contains at least two higher aliphatic hydrocarbon radicals, each having at least 11 carbon atoms, have their texture rendered soft and luxurious to the touch. Textiles such as cotton fabrics impregnated with these compounds as a rinse after washing are pleasingly soft and fluffy and give the appearance of being sun dried. The colloidally dispersible 1,2-substituted imidazolinium salts when added to the rinse water in small amounts after typical laundering operations impart a soft downy hand to the treated fabrics. Dosages in the rinse water can range from .001% to 1% by weight to a preferred treatment range of .005% to .01% by weight.

It has been the experience of the art that textile treatments must usually be water soluble to be effective. Water dispersible materials have been deemed imperfect for such operations as textile softening. Surprisingly, however, it has been discovered that while the water soluble imidazolinium salts were relatively ineffective as softeners and lubricants the colloidally dispersible 1,2-substituted imidazolinium salts gave superior results when employed for such purposes.

The expression "colloidally dispersible" refers to the character and physical appearance of aqueous suspensions containing 3% by weight of the 1,2-substituted imidazolinium salts. They range from milk white to light umber in color and vary in their viscosities from almost light cream to thick, rich viscous liquids. They may or may not be suspensions at the concentrations of use suggested herein.

The colloidally dispersible 1,2-substituted imidazolinium salts capable of use have the general formulae:

2



and

II-B:  $\left[ \begin{array}{c} \text{H} & + \\ | & | \\ \text{N} & \text{C} - \text{Y} \\ | & | \\ \text{R} - \text{C}_2 & \text{N} - \text{C} - \text{H} \\ | & | \\ \text{R}' & \text{D}' \text{R} \text{ Z \end{array} \right] \text{A}^-$

where D represents a divalent, non-amino organic radical containing less than 25 carbon atoms, composed of elements from the group consisting of C, H, O and N; D' represents a divalent organic radical containing less than 25 carbon atoms, composed of elements from the group consisting of C, H, O and N, and containing at least one amino group; R is a member of the class consisting of hydrogen and aliphatic and cycloaliphatic hydrocarbon radicals (e. g., cyclopentyl, cyclohexyl); R' is a member of the group consisting of alkyl, substituted alkyl (e. g., hydroxyalkyl such as  $\text{HOCH}_2\text{CH}_2$ ,  $\text{HOCH}_2\text{CH}_2\text{CH}_2$ , halo-alkyl such as  $\text{ClCH}_2\text{CH}_2$ ,  $\text{BrCH}_2\text{CH}_2$ ,  $\text{ClCH}_2\text{CH}_2\text{CH}_2$ —  
Br $\text{CH}_2\text{CH}_2\text{CH}_2$ —), and aralkyl radicals (e. g., benzyl, cinnamyl, etc.), with the proviso that at least two of the radicals R and R' contain at least 11 carbon atoms in an aliphatic chain; A represents an anion and is usually halide; Y and Z are hydrogen or a lower alkyl group containing not more than 6 carbon atoms.

A preferred species of compositions corresponding to the type illustrated in Formula II above has the structure:



wherein R is a member of the class consisting of aliphatic and cycloaliphatic hydrocarbon radicals and R' is a member of the group consisting of alkyl, substituted alkyl and aralkyl radicals, with the proviso that at least two of the radicals R and R' contain from 15 to 23 carbon atoms in an aliphatic chain, x is a small whole number, preferably 1 to 3, hal represents halide and n is an integer of 2 or more, preferably 2 to 6.

Examples of the 1,2-substituted imidazolines from which the imidazolinium compounds of the invention may be formed, are described in Wilson U. S. Patents 2,267,965 and 2,355,837. The imidazolines are usually formed by reacting an acid, and in the present instance preferably a fatty acid of at least 12 carbon atoms, with an alkylene polyamine (e. g., ethylene diamine, 1,2-propylene diamine) or a hydroxyalkyl alkylene polyamine (e. g., hydroxyethylethylene diamine) or a polyalkylene polyamine (e. g., diethylene triamine, triethylene tetramine, or tetraethylene pentamine). Some of the more readily available and preferred materials for preparing the starting imidazolines are the various fatty acids or mixtures of such acids as occur in various fats and oils and the polyamino compounds, diethylene triamine, tetraethylene pentamine and aminoethyl ethanolamine. Stearic acid and diethylene triamine when reacted to form 1-(2-aminoethyl)-2-heptadecyl imidazoline offers an excellent starting material. Another preferred imidazoline is 1-(2-hydroxyethyl)-2-heptadecyl imidazoline.

The additional long chain alkyl groups may be conveniently attached to the substituted radical in the 1-position of the preferred imidazolines by acylation or esterification.

I



fication with a suitable acid of appropriate chain length. Thus, 1-(2-aminoethyl)-2-heptadecyl imidazoline may be reacted with stearic acid under basic conditions to produce 1-(2-stearoylaminoethyl)-2-heptadecyl imidazoline, which is then quaternized with an alkylating agent, such as benzyl chloride, to produce the imidazolinium salt, 1-(2-stearoylaminoethyl)-2-heptadecyl-1-benzyl imidazolinium chloride.

In another preferred embodiment, an imidazoline formed from stearic acid and ethylene diamine, e. g., 2-heptadecyl imidazoline, is acylated with capric acid and then alkylated with octadecyl chloride to produce 2-heptadecyl, 1-decanoyl, 1-octadecyl imidazolinium chloride.

Other illustrative compounds that are colloidally dispersible in aqueous media and are useful in the practice of the invention are:

- (1) 1 - (2 - stearoxyethyl ethylstearate) - 2 - heptadecyl-1-methyl imidazolinium chloride.
- (2) 1 - (N - stearoylaminoethyl aminoethyl) - 2 - heptadecyl-1-ethyl imidazolinium bromide.
- (3) 1 - (2 - hydroxyethyl) - 2 - heptadecyl - 1 - octadecyl imidazolinium bromide.
- (4) 1 - (2 - palmitoylaminoethyl) - 2 - ethyl - 1 - hexadecyl imidazolinium chloride.
- (5) 1 - (2 - palmitoylaminoethyl) - 2 - heptadecyl - 1 - hexadecyl imidazolinium chloride.
- (6) 1 - (2 - stearoylaminoethyl) - 2 - heptadecyl - 1 - (2,3-hydroxypropane) imidazolinium chloride.
- (7) 1 - (2 - stearoylaminoethyl) - 2 - heptadecyl - 1 - propyl imidazolinium chloride.
- (8) 1 - (2 - stearoxyethyl) - 2 - heptadecyl - 1 - benzyl imidazolinium chloride.

In the above compounds the following alkylating agents were used in the preparation of the imidazolinium salts: (1) methyl chloride; (2) ethyl bromide; (3) octadecyl bromide; (4) hexadecyl chloride; (5) hexadecyl chloride; (6) 1-chloro-2,3-dihydroxy propane; (7) propyl chloride; and (8) benzyl chloride.

Any anion form of the imidazolinium salt other than halide may be employed. Sulfates, nitrates, nitrites, phosphates and carbonates produce useful treating agents.

It is thus apparent that long chain alkyl groups may be introduced into the 1,2-substituted imidazoline by a number of methods and at several places in the molecule.

Two interesting alkylating agents for the 1,2-substituted imidazolines have the following structural formulae:



Formula III is prepared by esterifying an alcohol with a halo-acetic acid to produce an ester. In Formula IV, halogen-2,3-hydroxy propane, produced by hydrolyzing an epihalohydrin, is esterified by an acid. In each case R is an aliphatic hydrocarbon radical and for the purposes of the invention preferably contains at least 11 carbon atoms.

When compositions III and IV are used to quaternize 1,2-substituted imidazolines, imidazolinium salts of the following generic formulae are produced:



wherein R, D, D', Y and Z have the significance shown in Formulae I and II, R' has the significance shown for R in Formulae III and IV and hal is a halide anion.

Specific examples of classes of compounds that fall within the above are shown below:



75 wherein each R above is an alkyl group and at least two

R's contain from 15 to 23 carbon atoms, and hal is a halide anion.

In a more preferred embodiment of compositions useful in the invention the R attached to the 2-carbon atom of the imidazolinium ring is a saturated 17 carbon atom alkyl group and each other R is a saturated 18 carbon atom alkyl group. Especially useful compositions are provided when only two of the possible three or more higher aliphatic hydrocarbon groups are long hydrocarbon chains. Thus the two compounds illustrated by the following structural formulae are highly suitable for use as textile softeners.

XIII



XIV



where R is an alkyl group containing from 15 to 23 carbon atoms.

In conducting numerous tests, it was found that the preferred species of colloidally dispersible 1,2-substituted imidazolinium salts contained only two saturated alkyl groups having from 15 to 23 carbon atoms. The compositions prepared from fatty acids or alcohols especially the saturated compounds, such as lauric acid, as well as the corresponding alcohols, are extremely useful. Stearic acid or stearyl alcohol give exceptionally good results.

In all of the foregoing chemical formulae one or more of the radicals R can also be an unsaturated hydrocarbon group. For example, at the 2-position the radical R can be the heptadecenyl radical which results when oleic acid is condensed with ethylene diamine, hydroxyethylmethylenediamine, diethylenetriamine, triethylenetetramine or tetraethylenepentamine to produce the imidazoline. Likewise, hydrocarbon radicals attached at the 1-position can be unsaturated. Thus, allyl chloride and other unsaturated quaternizing halides can be used instead of the saturated quaternizing agents previously described. In general, however, the best results are obtained when the aliphatic hydrocarbon chains of the R radicals are saturated.

In order to evaluate the compositions described above as textile softeners, the following test method was employed.

The test specimens were cotton diapers and cotton wash cloths which were indelibly numbered in one corner for purposes of identification. A portable 4-gallon, 1½ pound capacity washer and spin drier was used to treat from ¾ to 1 pound of fabrics. The specimens were washed three minutes in 4 gallons of Chicago tap water containing 75 cc. of a commercial anionic detergent. The water was drained and the test cloths spun dry for one minute. The washer was refilled with water to which had been added the treating chemical from an isopropanol suspension thereof. The rinse cycle was conducted for 3 minutes, the washer drained and the specimens again spin dried for 1 minute. Another similar rinse cycle was run on washed untreated specimens for purposes of comparison. Both the treated and untreated specimens were felt by at least 12 persons who gave their

opinions as to whether a treated specimen was soft and fluffy or whether it was relatively rough to the feel. The results of these tests were listed below in Table I. In these tests the specimens were room dried before testing.

Table I

|    | Composition                                                              | Percent by weight of treatment in rinse water | Percent of persons who found softness |
|----|--------------------------------------------------------------------------|-----------------------------------------------|---------------------------------------|
| 15 | 1. 1-(2-stearoylaminoethyl)-2-heptadecyl-1-benzyl imidazolinium chloride | .001<br>.05<br>.01<br>.1<br>0                 | 100<br>100<br>100<br>100<br>0         |
| 20 | 2.                                                                       | .001<br>.05<br>.01<br>0                       | 100<br>100<br>100<br>0                |
| 25 | 3. 1-(2-hydroxyethyl)-2-heptadecyl-1-benzyl imidazolinium chloride       | .001<br>.1<br>0                               | 0<br>8<br>0                           |
| 30 | 4. 1-(2-aminoethyl)-2-heptadecyl-1-octadecyl imidazolinium chloride      | .001<br>.001<br>.05<br>.01<br>0               | 100<br>100<br>100<br>100<br>0         |

Composition 3 was a water soluble compound and was ineffective in comparison with the other colloidally dispersible 1,2-substituted imidazolinium salts.

It is desirable to place the materials in a low molecular weight aliphatic alcohol such as isopropanol to prevent freezing during shipment. The higher dosages have the effect of making the fabrics treated soft and fluffy even after several subsequent washings without treatment. When dosages of about .05% to 1% by weight are used in the rinse operation, water repellency is imparted to the fabrics. If the user does not desire such an effect, treatments can be temporarily suspended or the dosage diminished until such effects are mitigated. In any event, simple experiments can determine optimum concentrations.

The compositions of the invention are relatively stable when prepared in an alcohol or water suspension but in the event separation occurs after a lapse of time, heating or agitation will restore the suspension to its original condition. Laboratory tests have shown fabrics treated in accordance with the invention will not yellow with age or with repeated treatment. The compositions are safe for home use when employed in the concentrations suggested herein.

The compositions of the invention are especially useful in treating hydratable fibers and cloth or sheets in which such fibers predominate, especially cellulose fibers such as cotton or blends of fibers in which cellulose predominates. The invention is also applicable to the treatment of wood fibers and cloth, glass fibers and cloth, and synthetic fibers and cloth made therefrom or made from blends of synthetic fibers and natural fibers, e. g., blends of Dacron (polyethyleneterephthalate) and wool, blends containing Orlon (acrylic fiber) and the like.

The treatment is especially advantageous where it is desired to overcome harshness of feel or to enhance softness to touch or to enhance water repellency of cloth or paper.

In all the compositions shown, the quaternization of the 1,2-substituted imidazolines is shown to be on the 1-nitrogen atom. This is believed to be correct. If, however, quaternization occurs at the 3-nitrogen atom such

is deemed an equivalency for the purpose of the invention. The invention is hereby claimed as follows:

The invention is hereby claimed as follows:

1. The method of treating cellulosic fibrous materials which comprises applying thereto an aqueous dispersion of a colloidally dispersible 1,2-substituted imidazolinium salt which contains at least two and not more than three higher aliphatic hydrocarbon radicals each having at least 11 carbon atoms, one of which higher aliphatic hydrocarbon radicals is in the 2-position of the imidazoline ring and another of which is in at least one of the 1-positions of the imidazoline ring and the cation radical.

2. The method of softening cotton textiles which comprises applying thereto an aqueous dispersion of a colloidally dispersible 1,2-substituted imidazolinium salt which contains at least two and not higher than three higher aliphatic hydrocarbon radicals each having at least 11 carbon atoms, one of which higher aliphatic hydrocarbon radicals is in the 2-position of the imidazoline ring and another of which is in at least one of the 1-position of the imidazoline ring and the cation radical

3. The method of softening textiles which comprises applying thereto an aqueous dispersion of a colloidally dispersible 1,2-substituted imidazolinium salt from the group consisting of



and



wherein DR together represents an ester and D'R represents an amide in which R in each instance is the acid portion and in which D represents a divalent, non-amino organic radical containing less than 25 carbon atoms, composed of elements from the group consisting of C, H, O and N; D' represents a divalent, organic radical containing less than 25 carbon atoms, composed of elements from the group consisting of C, H, O and N; R' is a member of the class consisting of hydrogen and aliphatic and cycloaliphatic hydrocarbon radicals; R is a member of the group consisting of alkyl, substituted alkyl and aralkyl radicals, with the proviso that at least two of the radicals R and R' contain at least 11 carbon atoms in an aliphatic chain; A represents an anion, and Y and Z are selected from the group consisting of hydrogen and a lower alkyl group containing not more than 6 carbon atoms.

4. The method of claim 3 wherein the 1,2-substituted imidazolinium salt is applied to the textiles from an aqueous medium containing from .001% to 1% by weight of said 1,2-substituted imidazolinium salt.

5. The method of claim 3 wherein the textile is predominantly cotton.

6. The method of softening textiles which comprises applying thereto a colloidally dispersible 1,2-substituted imidazolinium salt having the formula



wherein R is a member of the class consisting of aliphatic and cycloaliphatic hydrocarbon radicals and R' is a member of the group consisting of alkyl, substituted alkyl and aralkyl radicals, with the proviso that at least two of 75

the radicals R and R' contain from 15 to 23 carbon atoms in an aliphatic chain,  $x$  is a small whole number from 1 to 3 and hal represents halide and  $n$  is an integer from 2 to 6.

5 7. The method of claim 6 wherein the 1,2-substituted imidazolinium salt is 1-(2-stearoylaminoethyl)-2-heptadecyl-1-benzyl-2-imidazolinium chloride.

8. The method of claim 6 wherein the textile is predominantly cotton.

10 9. The method of softening textiles which comprises applying thereto the colloidally dispersible 1,2-substituted imidazolinium salt of the formula



10. The method of softening textiles which comprises applying thereto a colloidally dispersible 1,2-substituted 25 imidazolinium salt of the formula



wherein R is an alkyl group containing from 15 to 23 carbon atoms.

11. The method of softening textiles which comprises applying thereto a colloidally dispersible 1,2-substituted imidazolinium salt of the formula



wherein R is an alkyl group of at least 11 carbon atoms

12. A cellulosic fiber of the type used in textiles and  
5 paper impregnated with a minor amount of a colloidally  
dispersible 1,2-substituted imidazolinium salt which contains  
at least two and not more than three higher aliphatic hydrocarbon radicals each having at least 11 carbon atoms, one of which higher aliphatic hydrocarbon  
0 radicals is in the 2-position of the imidazoline ring and another of which is in at least one of the 1-position of the imidazoline ring and the cation radical

13. As a composition, a 1,2-substituted imidazolinium salt from the group consisting of



9

and



wherein DR together represents an ester and D'R represents an amide in which R in each instance is the acid portion and in which D represents a divalent, non-amino organic radical containing less than 25 carbon atoms composed of elements from the group consisting of C, H, O and N; D' represents a divalent organic radical containing less than 25 carbon atoms, composed of elements from the group consisting of C, H, O and N; R is a member of the class consisting of hydrogen and aliphatic and cycloaliphatic hydrocarbon radicals; R' is an alkyl radical; A represents anion and Y and Z are selected from the group consisting of hydrogen and a lower alkyl group containing not more than 6 carbon atoms.

14. A composition of the formula



wherein R is an alkyl group of at least 11 carbon atoms and hal represents halide.

15. A composition of the formula



16. A composition of the formula



wherein R is an alkyl group of at least 11 carbon atoms.

17. A composition of the formula



10

18. As a composition, a 1,2-disubstituted imidazolinium salt from the group consisting of



and



25 wherein DR together represents an ester and D'R represents an amide in which R in each instance is the acid portion and in which D represents a divalent non-amino organic radical containing at least 25 carbon atoms, composed of the elements from the group consisting of C, H, O and N; D' represents a divalent organic radical containing less than 25 carbon atoms composed of elements from the group consisting of C, H, O and N; R is a member of the class consisting of hydrogen and aliphatic and cycloaliphatic hydrocarbon radicals; R' is an alkyl radical; hal represents halide and Y and Z are selected from the group consisting of hydrogen and a lower alkyl group containing not more than 6 carbon atoms.

19. A composition of the formula



wherein R is an alkyl group containing from 15 to 23 carbon atoms.

20. A composition of the formula



60 wherein R is an alkyl group containing from 15 to 23 carbon atoms.

21. A composition of the formula



wherein R is an alkyl group containing from 15 to 23 carbon atoms.

75 (References on following page)

11

## References Cited in the file of this patent

## UNITED STATES PATENTS

|           |               |               |           |
|-----------|---------------|---------------|-----------|
| 901,009   | Imbert        | Oct. 13, 1908 | 2,267,965 |
| 2,031,603 | Holt          | Feb. 25, 1936 | 2,355,837 |
| 2,260,753 | Marple et al. | Oct. 28, 1941 | 2,493,322 |

12

|        |               |
|--------|---------------|
| Wilson | Dec. 30, 1941 |
| Wilson | Aug. 15, 1944 |
| Shonle | Jan. 3, 1950  |
| Weldon | Nov. 17, 1953 |
| Winsor | Jan. 10, 1956 |